

C. A. PFANSTIEHL.

PUPPET VALVE.

APPLICATION FILED FEB. 8, 1917.

1,393,726.

Patented Oct. 11, 1921.



Fig. 1



Fig. 4



Fig. 3

Fig. 5



Fig. 6



Fig. 7

Witnesses:

Albin C. Ahlberg.  
Chas. Pimbley

Inventor

Carl A. Pfanstiehl  
By William Bradbury, Jr.  
Attorneys.

# UNITED STATES PATENT OFFICE.

CARL A. PFANSTIEHL, OF HIGHLAND PARK, ILLINOIS, ASSIGNOR TO PFANSTIEHL COMPANY, INC., OF NORTH CHICAGO, ILLINOIS, A CORPORATION OF NEW YORK.

## PUPPET-VALVE.

1,393,726.

Specification of Letters Patent. Patented Oct. 11, 1921.

Application filed February 8, 1917. Serial No. 147,395.

To all whom it may concern:

Be it known that I, CARL A. PFANSTIEHL, a citizen of the United States, residing at Highland Park, in the county of Lake and 5 State of Illinois, have invented a certain new and useful Improvement in Puppet-Valves, of which the following is a full, clear, concise, and exact description, reference being had to the accompanying drawings, forming a part of this specification.

My invention relates to puppet valves for internal combustion engines.

The principal object of my invention is to provide a valve which shall be extremely 15 strong and at the same time light.

I accomplish my object by constructing my valve in accordance with the process set forth in my co-pending application Serial No. 276,044, filed February 10, 1919, for 20 improvement in articles of manufacture and method of making same.

In accordance with this co-pending application a valve is constructed having a pressed metal head of high speed steel fused 25 to a stem of a different character of steel more suitable for stems than is the high speed steel and also less-expensive.

In accordance with my present invention I fuse a hollow stem of so-called "Nychrome steel" to the central portion of a cupped disk of high speed steel and then fuse onto the other end of the stem a solid button of high carbon steel adapted to receive the thrust from the end of the push rod.

35 My invention is illustrated in the accompanying drawings in which,

Figure 1 represents a blank of high speed steel from which the valve head is constructed;

40 Fig. 2 represents the valve head pressed to form;

Fig. 3 illustrates the valve head and hollow stem in association with the supporting electrodes of a fusing machine before 45 the current is applied;

Fig. 4 represents the stem and valve in the fusing machine after the fusing operation;

Fig. 5 is a section through the rear re- 50 ceiving button;

Fig. 6 illustrates the valve stem and button in the fusing machine after the fusing operation; and

Fig. 7 represents the completed valve.

Similar characters of reference refer to 55 similar parts throughout the several views.

The high speed steel which I have found to be most desirable for valve heads contains besides its iron component, carbon .58%; phosphorus .01%; manganese, trace; 60 silicon .22%, tungsten 17.10%; chromium 4.5%, nickel .20%; and vanadium 1%. A disk 10 of this material is illustrated in Fig. 1, the preferred thickness being about  $\frac{1}{8}$  of an inch in the raw stock. This disk 65 may be punched, or otherwise cut, from sheets of annealed metal.

High speed or so-called tungsten steel which contains vanadium is worked only with great difficulty, but I have found that 70 by heating the disk to a temperature of between 1450 and 1550 degrees Fahrenheit the disk may be formed into the shape shown in Figs. 2 by a single operation. The heat must not be permitted to rise above 1550 75 degrees Fahrenheit because at greater temperature the metal when cooled by contact with the dies by means of which it is stamped becomes somewhat hardened. In fact so much so that it will not withstand 80 the irregular heat of the fusing operation without cracking. If, however the temperature to which the disk is raised for the stamping operation is maintained below 1550 degrees Fahrenheit the original annealed condition of the metal is not materially changed and the metal is not cracked by the heat of the fusing operation when the operation is carried on in the manner hereinafter described.

90 The disks 10, as illustrated in Fig. 2, are sandpapered, or otherwise brightened on both the upper and under sides of the central flattened portion and near the periphery on the concave side.

95 The stems which I have found most satisfactory for this type of valve are composed of what is termed "Nychrome steel." This steel analyzes substantially as follows in addition to its iron component: nickel 100 1.50%; chromium .35%; carbon .35%; manganese .50%; sulfur, less than .04%; phosphorous, less than .04%. Steel having this composition does not readily oxidize at the temperatures at which it is operated as valve 105 stems, nor is it seriously attacked by the combustion gases of an internal combustion engine. It withstands the wear incident to

the slipping up and down in the supporting sleeves better than either high speed steel or carbon steel.

In order to produce a valve in its finished form with a stem  $\frac{1}{8}$  of an inch in diameter I prefer to start out with a hollow stem about  $\frac{7}{8}$  of an inch outside diameter and provided with a  $\frac{1}{16}$  inch hole. In the completed valve, therefore, the thickness of the 10 wall of the valve stem is about  $\frac{1}{16}$  of an inch.

"Nychrome steel," such as I prefer to use for these valve stems, cannot be welded by the ordinary processes heretofore commonly used. This metal when heated to a temperature correct for the ordinary welding operation becomes so crumbly that if hit with a hammer it breaks up into small crystalline particles.

20 A tube 11 of metal of the above described character is clamped within the upper copper electrode 12 of an electric fusing machine. The disk 10 is supported upon the lower copper electrode 13 of the fusing machine. The electrodes 12 and 13 of this machine are connected with a suitable source of electricity sufficient for supplying a quantity of current about four times as great as that used in electric welding. The electrode 25 13 is so shaped that it initially contacts with the tungsten steel disk 10 only at or near the periphery of the disk, the purpose of this being to cause an initial flow of current radially through the disk to pre-heat the 30 latter at points away from the fusing position thereof in order to sufficiently soften the disk to prevent cracking due to the high heat of fusion and to prevent internal strains due to the cooling after the fusion 35 operation.

40 After assembling the disk 10 and stem 11 in the fusing machine a small inclosure 14 is brought into position about the parts to be united and hydrogen, or some other inert gas, is admitted to the space within the inclosure through the intake pipe 15. A downward pressure of several hundred pounds is now applied to the stem, but this pressure is insufficient to deflect the disk 10 45 so as to bring its central portion in contact with the lower electrode 13. While this pressure is still exerted the primary circuit of a transformer, which is preferably used for supplying the fusing current, is closed 50 and the current from the secondary is directed through the electrodes, the disk 10, and the stem 11. Although the circuit is completed for less than one second the result of the current flow is to heat the disk 10 55 throughout substantially its whole surface to a dull red thus softening it sufficiently that the disk is deflected under the pressure from the stem so that the lower central surface of the disk comes into intimate contact with the central portion of the lower elec-

trode. Immediately following this initial deflection of the disk the stem 11 begins to soften and melt away at the point of contact with the upper surface of the disk. The pressure is still maintained and the stem 70 is fed toward the disk as it melts away at its point of contact with the disk. After a movement of about one-half the distance through which the stem is fed against the disk the surface of the disk begins to melt 75 and thereafter throughout the remainder of the movement of the stem toward the disk the metal of the disk and that of the stem where they are gradually melted at the point of contact boils and bubbles and thoroughly 80 mixes. Some of this mixed metal is forced outwardly and forms the collar 16 shown in Fig. 4, while some of it is forced inwardly and ascends within the hollow portion of the tubular stem and forms the reinforcement 17 also shown in Fig. 4. This reinforcing portion 17 may be caused to ascend as much as three-fourths of an inch within the hollow portion of the tube if desired, but experiments show that a one-fourth inch rise of this reinforcing member carries the reinforcement beyond the point at which solid stems ordinarily give way under use and, therefore, that any further extension of this reinforcing member is 90 unnecessary. Analysis of the member 17 shows that the end most remote from the valve head is composed wholly of metal like the stem while portions nearer the valve head are composed of a mixture of the stem 100 and head metals.

105 Although the melting temperature for tungsten steel is several hundred degrees higher than that at which the stem metal melts, the herein described method of supporting the head and stem and of feeding the stem toward the head brings about the actual fluid condition of both head and stem at and near their points of contact, but at the same time maintains the other portions 110 of the head and stem so cool that the character of the metal is not changed at these other portions by the fusing operation. The surface of the head immediately opposite the point of fusion is kept so cool by 115 the copper electrode 13 that the mixture of the stem and head metals does not penetrate clear through to the under surfaces of the head 10. The collar of metal exuded from the stem and disk metals cools in contact 120 with the upper copper electrode 12 and thus forms a retainer for the molten interior metal preventing the latter from escaping during the final period of the fusion operation. In Fig. 4 the area of the blending 125 of the two metals is illustrated by the overlapping of the cross section lines of the stem and disk.

130 The metal most satisfactory for hollow stems is not satisfactory for receiving the

wear from the push rods and I have, therefore, found it advisable to fuse a button onto the end of the stem for receiving the wear. The button 18, shown in Fig. 5, is of the preferred form. This button may be made in a screw machine and is preferably made of high carbon steel. These buttons are preferably hardened by heating to red heat and then immersing in water. After being hardened they are placed in the same type of fusing machine as hereinbefore described and are fused by the same sort of operation as described in connection with the attachment of the head to the stem, excepting that the current required for fusing on the buttons is only about one-third that required for fusing together the heads and stems. The hardened buttons are supported in an electrode 19, as illustrated in Fig. 6, this electrode being of water cooled copper and making very intimate connection with the button 18. In this way the temperature of the button is maintained quite low and the temper is not drawn during the fusing operation. Before fusing the button onto the end of the stem the stem and head are brought each to its proper temper. The steel valve head at and very close to the margin of the fusion comes out of the fusion operation extremely hard and brittle. In order to prevent cracking of the disk around the fused portion the united members are annealed by packing in charcoal, or some other non-oxidizing packing, which excludes the air and by being held at a temperature between 1525 and 1550 degrees Fahrenheit for a period of one hour and then being gradually cooled down to about 200 degrees Fahrenheit throughout a period of two or three hours. When thus annealed all internal strains as were created during the fusing operation are permanently relieved. In order that the valves may be rotated for "grinding in" and for re-grinding during service a small slot 20, illustrated in Fig. 7, is milled into the base of the concave part of the head. The valves are then turned to within a few thousandths of the final size at which they are to be used in an ordinary lathe or a special machine. The machined valves, complete except for the attachment of the buttons 18, are then heated, preferably in an electric furnace, to a temperature of between 2000 and 2150 degrees Fahrenheit. It is desirable that the periphery of the valve head be hardened to a greater extent than is the central portion of the head. In order to accomplish this hardening of the

periphery it must be cooled more rapidly than the central portion of the disk and, in fact, more rapidly than the tubular stem because it is desirable that the stem itself be kept quite soft and tough. In order to satisfactorily cool the periphery of the disk I rotate the valve rapidly along the axis of the stem and at the same time apply a blast of cool air to the periphery of the head. I have found it desirable to protect the stem and central portion of the head from too rapid radiation and this may be done by any suitable inclosure.

After the head and stem have been hardened, as above described, the already tempered button 18 is fused to the stem in the manner hereinbefore described, care being taken to press the stem and button toward one another the right amount to secure a proper final length for the valve stem. The completed valve is lastly placed in a grinding machine and the head, stem, and button are ground to final size and finish.

Valves constructed in the manner herein described are particularly suitable for high speed engines since they have a strength substantially equivalent to valves having solid stems and uncupped heads. The amount of work required to oscillate the valves of high speed motors is no small proportion of the internal losses of the motors and by lightening the valves without material loss of strength a substantial proportion of the heretofore lost power may be recovered.

Having thus described my invention what I claim as new and desire to secure by Letters Patent of the United States is:

1. A valve for internal combustion engines comprising a hollow steel stem, a head fused thereto, the mixed metal of the head and stem extending into the hollow portion of the stem and reinforcing the latter at and near its union with the head.

2. A valve for internal combustion engines comprising a hollow steel stem, a head fused thereto, and means for reinforcing said stem at a point adjacent the union of the head and stem, comprising a block of metal formed integral with said head and extending into said stem.

In witness whereof, I hereunto subscribe my name this 31st day of January, A. D. 1917.

CARL A. PFANSTIEHL.

Witnesses:

ALBIN C. AHLBERG,  
CHAS. PIMBLEY.